

# UNITED STATES PATENT OFFICE.

CLEMENT L. PERKINS AND RALPH E. SAYRE, OF PITTSBURGH, PENNSYLVANIA,  
ASSIGNORS TO METALS RECOVERY COMPANY, OF NEW YORK, N. Y., A CORPO-  
RATION OF MAINE.

## FLOTATION OF MINERALS.

1,370,357.

Specification of Letters Patent.

Patented Mar. 1, 1921.

No Drawing.

Application filed July 13, 1920. Serial No. 395,999.

To all whom it may concern:

Be it known that we, CLEMENT L. PERKINS and RALPH E. SAYRE, citizens of the United States, residing at Pittsburgh, Allegheny county, State of Pennsylvania, have invented certain new and useful Improvements in the Flotation of Minerals; and we do hereby declare the following to be a full, clear, and exact description of the invention, such as will enable others skilled in the art to which it appertains to make and use the same.

This invention relates to the concentration of minerals, such as sulfid ores and the like, by flotation.

The invention is based upon the discovery that the flotation operation can, in many cases, be improved by the addition to the ore or mineral pulp of terpin hydrate. Terpin hydrate appears to have little if any selective action in bringing about the flotation of the mineral, but it has marked frothing qualities and provides an appropriate amount of froth with an ore pulp containing a suitable selective or collecting agent but lacking in frothing qualities, or with an ore pulp which requires no added selective agent but is lacking in frothing qualities. The terpin hydrate may thus be used to advantage with flotation agents which have marked selective or collecting properties but which are devoid of, or deficient in, frothing qualities.

The terpin hydrate can be incorporated with the ore or mineral pulp in any suitable manner which will insure its uniform incorporation and dissemination throughout the pulp. It may thus be incorporated by adding to the grinding mill, in which the ore is ground, or it can be added after the grinding operation and during or prior to the flotation operation. The flotation operation can be carried out in any suitable apparatus, such as an ordinary Callow cell, or in apparatus where the air is incorporated in the ore pulp by mechanical agitation.

It is of advantage in many cases, as with certain copper ores, to add to the ore pulp a small amount of alkali, which may be sufficient in amount to give to the ore pulp a distinct alkaline reaction. When alkalis are used, it is desirable to give them an appreciable time of contact with the ore pulp before subjecting the latter to flotation. The

alkalis can thus be added with advantage in the grinding mill so that they will be present during the grinding operation. The alkali may be caustic alkali such as sodium hydrate, or an alkaline salt, such as sodium carbonate, or even lime or calcium oxid or hydrate can be used.

The amount of the terpin hydrate added can vary somewhat, and may be as little as one-fifth of a pound per ton of ore (that is, calculated on the weight of the ore and not of the ore pulp). Larger amounts may, however, be used, as well as even smaller amounts in some cases.

The invention will be further illustrated by the following specific examples of tests made upon a copper sulfid ore:

Example 1: 500 parts by weight of Utah Copper Company's ore was ground in a pebble mill with 250 parts of water, lime equivalent to four pounds per ton of dry ore, and thiocarbanilid equivalent to one-fifth pound per ton. The ground pulp was transferred to a Calow rougher cell, diluted and floated after the addition of about 150 parts of water to which had been added terpin hydrate equivalent to one-tenth pound per ton of dry ore. A satisfactory froth was produced at once. Aeration of the pulp was continued until the concentration of the sulfid mineral practically ceased. A satisfactory concentrate and high recovery were obtained.

Example 2: The treatment was similar to that of Example 1, except that diazoamino-benzene equivalent to one-fifth pound per ton of dry ore was used in place of the thiocarbanilid.

With an ore of the character referred to in the above example, it is of importance to provide a selective or collecting agent to supplement the action of the terpin hydrate, which appears to be essentially that of a frothing agent with but little selective or collecting properties. Where, however, the ore pulp contains an appropriate selective or collective agent, or inherently requires the addition of no such agent but is deficient in frothing qualities, the addition of terpin hydrate, in a manner similar to that above described, imparts the desired frothing qualities, and provides bubbles in sufficient quantity and of sufficient persistency to overflow into the launder of the flotation

machine thereby mechanically facilitating the removal of the mineral concentrate.

It will be evident that, where selective or collecting agents are required, different agents may be used having the desired selective or collecting or mineral-modifying properties. Certain of these agents, such as thiocarbanilid and diazoaminobenzene, have very marked selective or collecting or mineral-modifying properties, but are substantially devoid of frothing qualities. The use of terpin hydrate, according to the present invention, is therefore of particular value in connection with the use of flotation agents of this character. The present invention can, however, be carried out with the use of other flotation agents, which may have both collecting and frothing qualities, but which are deficient in frothing qualities, and the requisite frothing properties can be imparted by the addition of the terpin hydrate, in a manner similar to that above described.

We claim:

1. The method of effecting the concentration of minerals by flotation, which comprises adding to the mineral pulp a small amount of terpin hydrate, and subjecting the resulting mixture to a flotation operation; substantially as described.

2. The method of effecting the concentration of minerals by flotation, which comprises adding to the mineral pulp a small amount of a selective or collecting or mineral-modifying agent, deficient in frothing qualities, together with a small amount of terpin hydrate, and subjecting the resulting mixture to a flotation operation; substantially as described.

3. The method of effecting the concentration of copper sulfid ores by flotation, which comprises adding to the mineral pulp a small amount of an alkali and a small amount of terpin hydrate, and subjecting the resulting mixture to a flotation operation; substantially as described.

4. The method of effecting the concentration of copper sulfid ores by flotation, which comprises adding to the mineral pulp a small amount of an alkali, a small amount of a flotation agent deficient in frothing properties, and a small amount of terpin hydrate, and subjecting the resulting mixture to a flotation operation; substantially as described.

In testimony whereof we affix our signatures.

CLEMENT L. PERKINS.  
RALPH E. SAYRE.